

3,232,762

**BROMOACYLURETHANS AS ANTIFOGGANTS**  
 John A. Ford, Jr., and Charles V. Wilson, Rochester, N.Y., assignors to Eastman Kodak Company, Rochester, N.Y., a corporation of New Jersey  
 No Drawing. Filed July 3, 1963, Ser. No. 292,762  
 13 Claims. (Cl. 96—109)

This invention relates to fog-inhibiting agents for photographic emulsions and to photographic emulsions containing them.

It is well known that photographic emulsions on storage tend to lose sensitivity and to become spontaneously developable without exposure to light. There is normally a detectable amount of the silver salt reduced during development in the areas where no exposure was given; this is commonly called "fog," and sometimes called "chemical fog" where it is necessary to distinguish between it and the effects of accidental exposure to radiation; in this invention we are not concerned with the latter.

Fog depends both on the emulsion and the conditions of development; for a given emulsion it increases with the degree of development. With constant development conditions, it tends to increase with time, temperature and relative humidity of storage conditions; it is common practice to make accelerated tests of the stability of photographic emulsions by storage at increased temperature or humidity, or both. It is, of course, desirable to have emulsions as stable as possible under the conditions of high temperature and humidity which may occur in tropical climates, for example. Fog usually appears over the whole area of the sensitive coating, but when severe, it is frequently non-uniform. Fog may also be caused by exposure to chemicals, for example, hydrogen sulfide and other reactive sulfur compounds, hydrogen peroxide vapor, and strongly reducing materials. While antifoggants may protect, to some extent, against such effects, it is normally understood that an antifogant protects against spontaneous growth of fog during prolonged storage or storage at high temperatures and humidities, or during development to maximum contrast and speed, or both.

It is, accordingly, an object of our invention to provide a new method for stabilizing photographic silver halide emulsions.

A further object is to provide novel photographic silver halide emulsions containing antifoggants or stabilizers.

It is another object of our invention to provide novel photographic silver halide emulsions that are stabilized with antifoggant addenda that do not objectionably desensitize the emulsions.

Other objects will become apparent from a consideration of the following description and examples.

According to our invention, photographic silver halide emulsions are stabilized with an alkyl bromoacylurethan. These compounds can be represented by the following general formula:



where  $n$  has a value of 1 to 7 inclusive, and R represents a member selected from the group consisting of an alkyl radical such as ethyl, butyl, octyl, etc. and a haloalkyl radical such as bromoethyl.

It has also been found in certain instances that a number of the compounds embraced by Formula I above serve to increase the sensitivity of photographic silver halide emulsions, in addition to stabilizing the emulsions or providing an anti-fog effect. However, the

fog-inhibiting effect is more general than the sensitizing effect, and for this reason, these compounds are referred to below as antifoggants or fog-inhibitors.

The fog-inhibitors of our invention can be added to the emulsion during the process of manufacture, either during mixing, ripening, or after-ripening, in order to avoid loss of sensitivity and/or to inhibit the growth of fog with the passage of time under non-ideal conditions of storage.

A solution of the compounds of the invention when added in suitable concentration, before coating, to unsensitized, chemically sensitized, or optically sensitized photographic emulsions may not appreciably affect the sensitometric values for sensitivity and fog when measurements are made soon after coating. Sensitometric measurements made at appreciable intervals of time, at elevated temperatures and dry or somewhat humid conditions show that these compounds do stabilize photographic speed and maintain fog at a low level.

The preparation of silver halide emulsions involves three separate operations: (1) the emulsification and digestion or ripening of the silver halide, (2) the freeing of the emulsion from excess soluble salts, usually by washing, and (3) the second digestion or after-ripening to obtain increased sensitivity. (Mees, "The Theory of the Photographic Process" (1952).) We prefer to add the fog-inhibiting agents after the final digestion or after-ripening, although they can advantageously be added prior to digestion. If desired, the fog-inhibiting agents of our invention can be incorporated in the emulsions without adverse effects by the bathing techniques known to those skilled in the art.

Listed below are a number of compounds coming within the scope of Formula I above which are typical of the antifoggants of our invention.



Many of the compounds embraced by Formula I above have been previously described in the prior art. These compounds can be prepared according to the procedure described by Johnson et al. in *J. Org. Chem.*, 25, 279-281 (1960). This method, briefly, comprises isomerizing N-bromosuccinimide to 3-bromopropionyl isocyanate which without isolation is treated with an alcohol to give the corresponding alkyl-3-bromopropionylurethan. Another method of preparing the antifoggants of this invention, given in *J. Org. Chem.*, 27, 3742 (1962), involves the reaction of oxalyl chloride upon an amide to form an acyl isocyanate which is again treated with an alcohol to form the corresponding acyl urethan.

The following specific examples illustrate these methods of preparation.

EXAMPLE 1

A mixture of 250 ml. of chloroform, 26.7 g. of N-nitrosuccinimide, 1 ml. of allyl chloride, and 5 mg. of benzoyl peroxide was refluxed with stirring for 4 hours. The resulting solution was cooled to room temperature, treated with a solution of 28.4 g. of 1-octadecanol in 100 ml. of chloroform and cooled overnight in a freezer. The solid which separated was filtered and dried. Recrystallization from ethyl acetate gave 28 g. of colorless crystals of octadecyl-3-bromopropionylurethan having a melting point of 97-98° C. This melting point agrees exactly with that reported in the literature [Johnson et al., J. Org. Chem., 25, 279, 280 (1960)].

EXAMPLE 2

A mixture of 11.7 g. of 6-bromocaproamide, 7.7 g. of oxalyl chloride, and 140 ml. of 1,2-dichloroethane was refluxed for 6 hours, cooled to room temperature, treated with 2.8 g. of ethanol, and allowed to stand overnight. The solid thus formed was filtered, and recrystallized once from ligroin and twice from cyclohexane to give 7.5 g. of colorless crystals of ethyl-6-bromocaprolylurethan having a melting point of 78-81° C.

*Analysis.*—Calcd. for  $C_9H_{16}BrNO_3$ : C, 40.6%; H, 5.02%. Found: C, 41.0%; H, 6.1%.

The photographic emulsions used in practicing our invention are generally of the developing-out type.

Various silver salts may be used as the sensitive salt in preparing the present emulsions such as silver bromide, silver iodide, silver chloride, or mixed silver halides such as silver chlorobromide, silver bromoiodide and the like.

In the preparation of the silver halide dispersions employed for preparing silver halide emulsions, there may be employed as the dispersing agent for the silver halide in its preparation, gelatin or some other hydrophilic colloidal material such as colloidal albumin, a cellulose derivative or a synthetic resin, for instance, a polyvinyl compound. Some colloids which may be used are poly(vinyl alcohol) or a hydrolyzed poly(vinyl acetate) as described in Lowe U.S. Patent 2,286,215, issued June 6, 1942.

The emulsions of the invention can contain conventional photographic silver halide emulsion addenda such as optical sensitizers, chemical sensitizers, coating aids, gelatin hardeners, plasticizers, and the like, as well as other antifoggants in conjunction with the present antifoggants.

The present photographic emulsions of the invention can be coated on any of the conventional photographic

supports including paper, cellulose acetate film, polyethylene film, polyethyleneterephthalate film, polystyrene film, glass and the like.

The optimum amount of fog-inhibiting agent can be determined by making the customary tests employed in emulsion making. Of course, the optimum amount for a given emulsion will vary depending on the presence of emulsion addenda, such as chemical sensitizers, optical sensitizers, etc. In general we have found that from about .01 to about 20 g. of fog-inhibiting agent per mole of silver halide is suitable for the purpose of our invention, with a preferred range of from about .1 to about 10 g. of fog-inhibiting agent per mole of silver halide. Instead of adding the fog-inhibiting agent directly to the photographic emulsion, it is sometimes desirable to incorporate the fog-inhibiting agent in a separate water-permeable hydrophilic colloid layer which is contiguous with the silver halide emulsion layer which is to be stabilized. In such embodiments of the invention we prefer to use the higher concentrations of fog-inhibiting agents.

The present invention is further illustrated by the following examples of preferred embodiments thereof. In the following examples the stabilizing action of several typical antifoggants of the invention in silver halide emulsions was determined by incubation of the emulsion for two weeks at a temperature of 120° F. and constant relative humidity of about 50-55 percent. The efficiency of the various tested antifoggants was determined by measuring the speed, gamma and fog of the incubated emulsions containing an antifoggant and comparing these measurements with those of the same batch of emulsion before incubation. Also, similar measurements were made with a photographic emulsion containing no antifoggant both before and after incubation. The tests were made using high speed, negative-type silver bromo-iodide emulsions (coated on cellulose acetate supports), which had been panchromatically sensitized with cyanine dyes. The test films were exposed on an intensity scale sensitometer (Kodak Type Ib) and developed for 5 minutes at 68° F. in the following composition:

|    |                                | Gms. |
|----|--------------------------------|------|
|    | p-Methylaminophenol sulfate    | 2.5  |
|    | Sodium sulfite, desiccated     | 30.0 |
| 45 | Hydroquinone                   | 2.5  |
|    | Sodium metaborate, octahydrate | 10.0 |
|    | Potassium bromide              | 0.5  |
|    | Water to make 1 liter.         |      |

The speed, gamma and fog for each of the emulsion coatings were then measured as indicated above. The results obtained are given in the following tables.

Table I

| Example  | Compound No. | Concentration, gms./mole AgX | Fresh Coatings |       |      | Incubated Coatings |       |      |
|----------|--------------|------------------------------|----------------|-------|------|--------------------|-------|------|
|          |              |                              | Speed          | Gamma | Fog  | Speed              | Gamma | Fog  |
| (a)----- | Control      | -----                        | 100            | 0.90  | 0.10 | 65                 | 0.73  | 0.28 |
| (b)----- | 1            | 3.0                          | 100            | 0.97  | 0.11 | 85                 | 0.90  | 0.10 |
| (c)----- | 6            | 3.0                          | 120            | 1.03  | 0.10 | 94                 | 0.90  | 0.15 |
| (d)----- | 6            | 6.0                          | 110            | 0.95  | 0.10 | 83                 | 0.82  | 0.11 |

Table II

| Example  | Compound No. | Concentration, gms./mole AgX | Fresh Coatings |       |      | Incubated Coatings |       |      |
|----------|--------------|------------------------------|----------------|-------|------|--------------------|-------|------|
|          |              |                              | Speed          | Gamma | Fog  | Speed              | Gamma | Fog  |
| (e)----- | Control      | -----                        | 100            | 1.20  | 0.11 | 35                 | 0.80  | 0.49 |
| (f)----- | 2            | 3                            | 97             | 1.27  | 0.11 | 60                 | 0.97  | 0.16 |
| (g)----- | 2            | 6                            | 95             | 1.23  | 0.10 | 62                 | 1.05  | 0.10 |
| (h)----- | 3            | 3                            | 95             | 1.28  | 0.10 | 67                 | 1.02  | 0.10 |
| (i)----- | 3            | 6                            | 85             | 1.27  | 0.10 | 50                 | 0.97  | 0.07 |
| (j)----- | 4            | 3                            | 97             | 1.30  | 0.10 | 62                 | 1.08  | 0.12 |
| (k)----- | 4            | 6                            | 87             | 1.12  | 0.09 | 52                 | 0.88  | 0.08 |
| (l)----- | 5            | 3                            | 100            | 1.25  | 0.10 | 48                 | 1.00  | 0.21 |
| (m)----- | 5            | 6                            | 100            | 1.25  | 0.09 | 58                 | 1.07  | 0.09 |

We claim:

1. A photographic silver halide emulsion containing an alkyl(monobromoalkanoyl)urethan antifoggant.
2. A photographic silver halide emulsion containing an antifoggant compound having the formula:



wherein  $n$  is an integer of 1 to 7 and R is an alkyl radical.

3. A photographic silver halide emulsion containing an antifoggant compound having the formula:



wherein R is an alkyl radical having 1 to 18 carbon atoms.

4. A photographic gelatino silver halide developing-out emulsion containing from about .01 g. to about 20 g. per mole of silver halide of an antifoggant having the following formula:



5. A photographic gelatino silver halide developing-out emulsion containing from about .01 g. to about 20 g. per mole of silver halide of an antifoggant having the following formula:



6. A photographic gelatino silver halide developing-out emulsion containing from about .01 g. to about 20 g. per mole of silver halide of an antifoggant having the following formula:



7. A photographic gelatino silver halide developing-out emulsion containing from about .01 g. to about 20 g. per

10

15

20

25

30

35

40

6  
mole of silver halide of an antifoggant having the following formula:



8. A photographic gelatino silver halide developing-out emulsion containing from about .01 g. to about 20 g. per mole of silver halide of an antifoggant having the following formula:



9. A photographic gelatino silver halide developing-out emulsion containing from about .01 g. to about 20 g. per mole of silver halide of an antifoggant having the following formula:



10. A photographic element comprising a photographic silver halide emulsion layer and a contiguous water-permeable hydrophilic colloid layer, at least one of said layers containing an alkyl(monobromoalkanoyl)urethan.

11. A photographic silver halide emulsion as described in claim 2 wherein the silver halide is silver bromoiodide.

12. A photographic silver halide emulsion as described in claim 2 wherein the R substituent of the antifoggant compound is a haloalkyl radical.

13. A photographic silver halide emulsion as described in claim 3 wherein the R substituent of the antifoggant compound is a bromoalkyl radical having 1 to 18 carbon atoms.

#### References Cited by the Examiner

#### UNITED STATES PATENTS

2,944,902 7/1960 Carroll et al. ----- 96—107

#### OTHER REFERENCES

J. Org. Chem., vol. 25, pages 279—291 (1960).

J. Org. Chem., vol. 27, pages 3742 and 3743 (1962).

NORMAN G. TORCHIN, Primary Examiner.